

[54] **COLORING HYDROPHOBIC FIBERS USING CARRIER OF HALOGENATED HYDROXYBIPHENYLETHER**

[75] Inventors: **Kurt A. Dellian, Spring Valley; Thomas A. Furia, Hartsdale, both of N.Y.**

[73] Assignee: **Ciba-Geigy Corporation, Ardsley, N.Y.**

[22] Filed: **Mar. 6, 1972**

[21] Appl. No.: **232,191**

[52] U.S. Cl. .... **8/173, 260/613 R**

[51] Int. Cl. .... **D06p 5/04**

[58] Field of Search ..... **8/173; 260/613 R**

[56]

**References Cited****UNITED STATES PATENTS**

|           |        |                    |           |
|-----------|--------|--------------------|-----------|
| 2,270,706 | 1/1942 | Heymann .....      | 8/173     |
| 3,385,652 | 5/1968 | Walter et al ..... | 8/173 X   |
| 3,506,720 | 4/1970 | Model et al .....  | 260/613 R |

*Primary Examiner*—Thomas J. Herbert, Jr.  
*Attorney, Agent, or Firm*—Mr. Joseph G. Kolodny;  
Mr. Stanley A. Marcus; Dr. E. McC Roberts

[57]

**ABSTRACT**

Organic hydrophobic fibers are colored using a disperse or cationic dyestuff employing a carrier component of a halogenated hydroxybiphenylether.

**6 Claims, No Drawings**

**COLORING HYDROPHOBIC FIBERS USING  
CARRIER OF HALOGENATED  
HYDROXYBIPHENYLETHER**

**BACKGROUND OF THE INVENTION**

The present invention is directed to a process for coloring as through dyeing or printing hydrophobic organic polymer fibers employing an additional carrier component.

It is well known in the prior art techniques of dyeing and printing that special procedures are necessary to color a textile structure of fabric that is essentially water impermeable since otherwise serious problems arise. For example, with many conventional techniques, the dyestuff does not penetrate the water impermeable material and does not affect coloration. In the event coloration does occur, it is not permanent and leaches out during subsequent washing steps.

To circumvent the problems of the noncoloration or the leaching of the dye, the prior art has employed in the treatment of the hydrophobic synthetic fibers elevated pressures with temperatures greater generally than 250° F. Generally speaking, dyeing under pressure at elevated temperature is undesirable due to expensive and complex procedures. To bypass this dyeing technique, the prior art has also turned to specific carrier components. These carriers aid in the penetration of the dye into the fiber by causing a swelling of the base substrate.

The use of carriers in dyeing techniques upon hydrophobic fibers allows satisfactory results at temperatures as low as 200° to 210° F although a temperature of 212° F at normal atmospheric pressure is preferred. There are many carrier components for hydrophobic fibers known in the prior art to be employed with a variety of dyes. Among the typical carriers used by the art up to the present time are various derivatives of benzene and phenol such as ortho- and para-phenylphenol, chlorinated benzenes, xylenes, naphthalenes, toluenes, aromatic esters or ethers, and biphenyl. Nevertheless many of these carrier components have some drawbacks such as lack of availability, undue toxicity, lack of ease of removal from the substrate, effect on lightfastness of color, or influence of buildup of a heavy shade.

It is an object of this invention to provide a novel carrier component which is suitable for dyeing hydrophobic material.

**DESCRIPTION OF THE INVENTION**

The method of the invention employs a disperse or cationic dyestuff in dyeing or printing hydrophobic organic fibers. In conjunction with the dyestuff a carrier component is employed which adds the penetration of the dyestuff into the substrate material.

Accordingly in the present technique of this invention, dyeing and printing of synthetic hydrophobic fiber using a disperse or cationic dyestuff is undertaken with an emulsion or dispersion of a carrier component of a halogenated hydroxybiphenylether. This carrier is of the following formula:



wherein

X is halogen,

n is an integer from 0 to 3,

Y is chlorine or bromine,

m is an integer from 0 to 3,

the sum of n and m is 1 to 3.

A preferred class of compounds within the above definition is when X and Y are specific to chlorine.

The carriers of this invention of the halogenated hydroxybiphenylether type are found in U.S. Pat. No. 3,506,720 issued Apr. 14, 1970. The disclosure of this patent is incorporated by reference herein.

The carrier compounds of the present invention are, in most cases, clear colorless solids. They are utilized in the form of an emulsion or dispersion composition which is added to the dyebath formulation, printing paste, or prescouring bath. Besides the carrier activity they possess a bacteriostatic action.

The carriers of the present invention are generally colorless, odorless and non-toxic, or nearly so. They usually do not affect the fastness other than by improving it, and are either non-foaming or very low foaming. Dyeing processes utilizing the carrier composition of the present invention exhibit a slow drawing of the dyestuff resulting in excellent levelness and extremely good utilization or exhaustion of the dyestuff.

The types of dyestuffs employable in the present invention are well known in the art as disperse and cationic dyestuffs. Illustrative although not limiting of suitable disperse dyestuffs are those listed in the Color Index under the Disperse dye classification.

There are various techniques and procedures for dyeing the synthetic fibrous material utilizing the disperse or cationic dyestuff and carrier component disclosed herein. As employed herein, a fabrous material includes fibers, yarns, threads, fabric ribbons, tapes and tabs.

The dyestuff and emulsified carrier may be added to a bath at temperature equivalent to the boiling point of water. A time interval of two or three hours is utilized during which time the fibrous substrate is contacted with the dyebath composition. Thereafter the fabric is washed followed by drying.

Another technique of applying the dyestuff in emulsified carrier with a composition containing the dyestuff carrier and emulsifying agent which is applied by padder on the substrate followed by steaming for a time period of 10 of 15 minutes.

Insofar as printing techniques are concerned printing may be carried out in the usual way by adding the carrier emulsion to a paste and printing the material on a roller or screen printing unit followed by fixing the dye by exposing to steam or heat treatment.

A thermosol technique may be utilized by padding the material with a mixture of a disperse dye-emulsified carrier of the type disclosed herein followed by drying at 100° to 250° C for 1 to 30 minutes. Alternatively thermofixing may take place with steam injection at temperature-time conditions as 340° F for 1 to 30 minutes.

The types of substrates that may be employed as previously disclosed are hydrophobic materials that do not color readily without the use of a carrier component.

Suitable examples of the hydrophobic material include



## EXAMPLE 2

The procedure of Example 1 is repeated but employing 3 parts by weight of the fiber of a dyestuff of the formula:



A strong reddish brown shade of excellent light fastness is obtained.

## EXAMPLE 3

A printing paste is prepared containing 10 parts of the carrier composition described in Example 1, 2.5 parts of a dyestuff of the formula:



3 parts sodium alginate thickener, and 20 parts mineral spirits. A polyethylene terephthalate cloth is printed with the paste and then the printed cloth is cured for 1 minute at 350°-90° F. The cloth is then soaped and rinsed. A vivid reddish blue shade is obtained.

## EXAMPLE 4

Following the general procedure of Example 1, a fabric of acid modified polyethylene terephthalate (Dacron 64) is dyed using 1.5 parts of a dyestuff of the formula:



However, this procedure employs ethoxylated nonylphenol in place of the sodium salt of oleyl amylester sulfate. A brilliant pink shade having good fastness properties is obtained.

## EXAMPLE 5

The procedure of Example 1 is repeated but employing 2.5 parts of the dyestuff of the formula:



and 6 parts of the carrier emulsion composition. A vivid pink shade of excellent fastness is obtained.

## EXAMPLE 6

5 A dye carrier composition is prepared in like manner as Example 1, but instead of 2 hydroxy - 2',4, 4' - trichlorodiphenylether, 2 hydroxy - 4,4' dichlorodiphenylether is used. In this example, the following dyestuff 10 is added:



15 20 A liquor ratio of 40:1 is present in the dye bath with 100 pounds of polyethylene terephthalate (Dacron 54) fabric. Initially the bath temperature is at 140° F followed by raising the temperature to boiling over a period of 20 minutes which is maintained for 90 minutes. 25 The fabric is rinsed, soaped, and placed in a bath of 2% hydrosulfite and 2% weight soda ash for 15 minutes at 180° F. A brilliant yellow shade having excellent fastness properties results.

## EXAMPLE 7

30 A dye carrier emulsion is prepared in similar fashion as Example 1. The carrier powder of a weight concentration is added at 85° C to a blank dyebath without dyestuff containing Dacron Knit material in a liquor 35 ratio of 40:1.

35 The temperature is raised over a 3 minute period to boiling which is maintained for another 30 minutes. The blank dyebath is then dropped. Thereafter the Dacron Knit material is dyed in a new bath containing 3% (owf) of the following dyestuff:



45 50 With the dyebath keep at boiling, the dyeing proceeds for a period of 60 minutes. The fabric is rinsed and treated with hydrosulfated soda ash, soaped and again rinsed. A deep brown shade having excellent fastness properties is obtained.

## EXAMPLE 8

55 The procedure of Example 6 is repeated but employing the dyestuff of the formula:



65 A very deep orange shade results.

## EXAMPLE 9

The procedure of Example 1 is repeated but employing instead of 2 hydroxy 2',4, 4' - trichlorobiphenyl-ether, 2 hydroxy - 4' chloro biphenyl ether. Additionally, the following dyestuff is substituted.



A blue shade of good fastness results.

## EXAMPLE 10

The procedure of Example 1 is repeated but using a mixture of the following dyestuff are employed at equal concentrations:



A brilliant violet shade of excellent fastness results.

## EXAMPLE 11

The procedure of Example 1 is repeated in all essential respects but instead of Dacron, a fabric of Nylon 66 (polyamide) is used.

A strong shade of yellow is obtained.

What is claimed is:

1. In a process for coloring fibrous material selected from the group consisting of polyester, polyamide, polypropylene, polyacrylonitrile and triacetate with a disperse or cationic dyestuff with the aid of a carrier component in an emulsion or dispersion, the improvement comprising utilizing a carrier component of the following formula:

10



15

wherein

X is halogen,

n is an integer from 0 to 3,

Y is chlorine or bromine,

m is an integer from 0 to 3,

the sum of n and m is 1 to 3.

2. The process of claim 1 wherein said halogen is chlorine or bromine.

3. The process of claim 2 wherein said halogen is chlorine.

4. The process of claim 1 wherein both X and Y represent chlorine.

5. The process of claim 1 wherein said fibrous material is a polyester.

6. The process of claim 1 wherein said fibrous material is a polyamide.

\* \* \* \* \*

40

45

50

55

60

65